

## UNITED STATES PATENT OFFICE

HAROLD ROBERT RAFTON, OF LAWRENCE, MASSACHUSETTS, ASSIGNOR TO RAFFOLD PROCESS CORPORATION, A CORPORATION OF MASSACHUSETTS

## METHOD OF IMPROVING PAPER MACHINE OPERATION

No Drawing. Application filed December 11, 1928, Serial No. 325,408. Renewed March 5, 1931.

This invention relates to the manufacture of paper and more particularly to the manufacture of paper filled with alkaline filler.

The principal object of my invention is to provide a method for paper manufacture whereby alkaline filler furnishes may be run on the paper machine substantially free from soft lumps.

An important object of my invention is to provide a method whereby both alkaline filler and casein may be used in the same furnish substantially without difficulty from soft lump formation.

A further object of my invention is to produce paper containing both casein and alkaline filler, which is substantially free from lumps and lump spots.

Other objects and advantages of my invention will become apparent during the course of the following description.

In the manufacture of substantially unsized paper filled with alkaline filler, particularly when old paper stock is one of the fibrous constituents, soft lumps form in the furnish and cause breaks on the paper machine. I have found that this formation of lumps is traceable to the presence in the furnish of casein from "coated broke", and that the trouble from soft lumps may be substantially eliminated in the manufacture of paper filled with alkaline filler by substantially excluding casein from the furnish. However this exclusion is not always feasible or desirable.

In my copending application Serial No. 325,407, filed December 11, 1928, I disclose a method whereby the manufacture of paper filled with alkaline filler may be carried on substantially free from soft lumps or at least with only a commercially unimportant number of soft lumps even in the presence of casein in the furnish. It is to be noted that the casein which is present finds its way into the furnish from the coated "broke" (this term including the coated paper present in clippings, trimmings, or the like) in the furnish, or from the old paper stock made from old papers possessing some casein bearing constituents, or from circulating mill waters which in turn originally derive their casein

from such sources, or even from casein added directly to the furnish. In the method disclosed in my last mentioned copending application, alum is added at the wet end of the paper machine to a furnish which contains casein, and thereby soft lumps are substantially avoided. In the present application I disclose another method for accomplishing this same result.

The method I employ is similar to that which I disclose in my copending application Serial No. 304,167, filed September 5, 1928, and Serial Nos. 321,753 and 321,754, both filed November 24, 1928. It consists substantially in adding alkaline filler, preferably continuously, preferably in suspension, at the wet end of the paper machine to a mix including fibrous material, casein, and alum, and sizing materials if such are to be used.

In the preferred practice of my invention I add to the beater or other similar machine all fibrous materials to be used, with the exception of those fibrous materials coming under the definition of alkaline filler herein-after set forth and such fibrous material as is present in the stock recovered from the white water. The casein bearing constituent which is normally a part of the fibrous furnish is also added in the beater. I may also add to the beater alum, or rosin size and alum, or sodium silicate and alum, or both rosin size and sodium silicate and alum. In any event, I prefer to have an excess of alum present. Filler other than alkaline filler may be added if desired as well as coloring matter or the like.

After the usual treatment in the beater, the mix is preferably passed through the beater chest, jordan, and machine chest in the customary manner. This procedure and/or order of steps is not essential, and may vary considerably as will be apparent to one skilled in the art. The mix, still in relatively concentrated form, is now at the point where it is ready for dilution preparatory to delivery to the web-forming end of the paper machine. All water used for dilution up to this point in the process is preferably either fresh water, or white water which has been purified so that it contains only a negligible amount of

alkaline filler. However, at this point, untreated white water as obtained from the paper machine may be used as diluting water. During dilution at this point, or subsequent thereto, the alkaline filler preferably in aqueous suspension is added preferably continuously, due care being taken that adequate mixing is insured.

According to the definition of alkaline filler hereinafter set forth, this term includes fibrous matter in combination with the mineral alkaline filler itself. In such cases the fibrous material must be properly broken down in a suitable apparatus before addition, as will be apparent. It may be refined separately if desired, but ordinarily this will be unnecessary as such fibres have already been once refined in the previous papermaking procedure.

Moreover, the stock recovered from the white water contains alkaline filler and this stock preferably should not be added at a point prior to the point of dilution preparatory to delivery to the web-forming end of the paper machine as the content of alkaline filler would tend to injure or destroy the effect desired because of the relatively prolonged contact in a relatively concentrated condition.

Moreover, the recovery of the stock from the white water should take place as soon as possible after the production of the white water and such stock should preferably be returned promptly to its point of re-use so as to afford as little time as possible for contact between the alkaline filler and the constituents of the mix which have accompanied it in the white water.

If the recovered stock be obtained from a settling system, a convenient way is to add the recovered stock directly from this settling system continuously at the mixing box at the point of dilution of the stock. If the stock is recovered by a filter or deckering system by mixing the white water with relatively concentrated stock as a "sweetener," then a convenient method is to divert part or all of the stream of concentrated fibrous stock just before its delivery to the mixing box, and utilize this as "sweetener" stock, delivering it after it has so functioned to the mixing box. In this way the stock containing the alkaline filler derived from the white water remains for only a brief interval in concentrated condition, and is quickly diluted at the mixing box.

Where casein containing constituents are to be used, in order to prevent soft lumps the alkaline filler must be added as stated above at or subsequent to the point where the stock is in dilute condition; if it be added prior to this point, it results in the production of soft lumps in the mix. In order to have my method effective, the alkaline filler must be added at a point where there is a minimum of

intimacy and time of contact of the alkaline filler with the constituents of the mix. The intimacy of contact is particularly damaging at high concentrations, particularly when accompanied by agitation. When the intimacy and time of contact are reduced to a minimum, as they are at the wet end of the paper machine, the tendency for the alkaline filler in conjunction with the casein bearing constituent to form soft lumps is greatly reduced if not entirely eliminated.

An illustrative furnish which may be satisfactorily used in carrying out my invention is as follows:

| <i>Materials added in beater</i>                                                       | Pounds |
|----------------------------------------------------------------------------------------|--------|
| Fibrous furnish, e. g. sulphite pulp and soda pulp, equal parts (air dry weight) ----- | 1400   |
| Casein containing ingredient (air dry weight), e. g. coated "broke" -----              | 300    |
| Alum -----                                                                             | 40     |

*Material added proportionately and continuously on dilution*

|                                                                                      | Pounds |
|--------------------------------------------------------------------------------------|--------|
| Alkaline filler (bone dry weight), e. g. calcium carbonate magnesium hydroxide ----- | 300    |

Another furnish which may be used is:

| <i>Materials added in beater</i>                                                                        | Pounds |
|---------------------------------------------------------------------------------------------------------|--------|
| Fibrous furnish, e. g. sulphite pulp, soda pulp and old paper stock, equal parts (air dry weight) ----- | 1400   |
| Casein containing ingredient (air dry weights) e. g. coated "broke" -----                               | 300    |
| Rosin size -----                                                                                        | 6      |
| Alum -----                                                                                              | 60     |

*Material added proportionately and continuously on dilution*

|                                                                                      | Pounds |
|--------------------------------------------------------------------------------------|--------|
| Alkaline filler (bone dry weight), e. g. calcium carbonate magnesium hydroxide ----- | 300    |

Another furnish which may be used is:

| <i>Materials added in beater</i>                                                                        | Pounds |
|---------------------------------------------------------------------------------------------------------|--------|
| Fibrous furnish, e. g. sulphite pulp, soda pulp and old paper stock, equal parts (air dry weight) ----- | 1400   |
| Casein containing ingredient (air dry weight) e. g. coated "broke" -----                                | 300    |
| Rosin size -----                                                                                        | 60     |
| Alum -----                                                                                              | 100    |

*Material added proportionately and continuously on dilution*

|                                                                                     | Pounds |
|-------------------------------------------------------------------------------------|--------|
| Alkaline filler (bone dry weight) e. g. calcium carbonate magnesium hydroxide ----- | 300    |

The furnishes given above are to be considered as illustrative only and not limiting, as I have found that I may carry on my

invention with a wide variety of materials used in widely varying quantities and still obtain satisfactory results.

It will be noted in the second illustrative furnish given above, that the rosin size is present in an amount of six pounds in a total furnish of approximately 2000 lbs., or approximately only three-tenths of one per cent. on the total furnish. As is apparent, this is an amount of size insufficient to impart a substantial degree of sizing to the paper. Its use in that furnish is thus obviously not from the standpoint of sizing the sheet, but rather for the purpose, well known in the art, of imparting better running qualities to the stock on the paper machine.

The papers made by my process may be finished as usual as by machine calendering or supercalendering if desired, and if sized, may be used for conversion, e. g. for coating.

My method is particularly valuable as it permits the operation of a mill manufacturing both coated paper and alkaline filled paper without the segregation of the coated "broke" into furnishes which do not contain alkaline filler. It also does away substantially with the difficulties and necessity of isolating casein bearing ingredients from alkaline filler furnishes.

I have found that it is particularly advantageous to combine the methods disclosed in my copending application Serial No. 325,407, filed December 11, 1928, with that disclosed in the present application, namely, when casein bearing constituent is used in the mix, to add both the alkaline filler and the alum at the wet end of the paper machine. The chief advantages of this combined process are that the "broke" containing alkaline filler may thereby be used directly in the beater, and that the capacity of the beater for fibrous material, and its beating efficiency, are enhanced by the absence of the major part of the filler from the beater. Furthermore the material recovered from the white water which of course contains alkaline filler may thereby be delivered to the beater or at any other point where the stock is still in concentrated condition, such as for instance in any of the stuff chests. This procedure permits the utilization of the equipment commonly used for white water recovery with the normally employed piping connections, instead of the changed piping required when only the alkaline filler is added at the wet end of the paper machine. Where the recovery system is of the filtering or deckering type, the "sweetener" stock may be taken exactly as is customary from one of the stuff chests, and this stock together with the recovered material from the white water may be returned thereto or elsewhere in the concentrated stock system as desired. A method similar to this method is broadly claimed in my copending application Serial No. 321,754, filed Novem-

ber 24, 1928, but the specific use of that method when casein is employed in the furnish, or the advantages inherent thereto, namely, the substantial elimination of soft lumps, is not therein disclosed.

In the place of alum, I may use with a measure of success certain acidic materials such as sulphuric acid ( $H_2SO_4$ ), or acid salts such as sodium bisulphate ( $NaHSO_4$ ), or metallic salts such as zinc sulphate, or other salts of aluminum such as the chloride or the like. Because of economy, however, I prefer to use ordinary alum.

In place of rosin size I may use other sizes, such as soaps, for example the oleates, or any other material derived by treatment with an alkaline substance or the like from material originally of acid characteristics or from material which likewise is of a partly or completely saponifiable nature such for example as saponified beeswax. I may also use other sizing materials such as paraffin emulsions, for example as set forth in my copending applications Serial Nos. 304,170, 304,173, 304,176 and 304,177, all filed September 5, 1928.

Where I use the term "alkaline filler," I mean substantially water insoluble filler which when agitated in contact with freshly boiled distilled water, say for an hour, will impart a pH value to such water greater than 7.0 that is, which will be on the alkaline side of the neutral point. Among the fillers included in this group may be mentioned calcium carbonate, of which lime mud from the causticizing process is one form; calcium carbonate magnesium basic carbonate employed in the paper disclosed in my U. S. Patent No. 1,595,416, issued August 10, 1926; calcium carbonate magnesium hydroxide disclosed in my U. S. Patent No. 1,415,391, issued May 9, 1922; and other substantially water insoluble normal or basic carbonates of alkaline earth metals (which expression is herein intended to include magnesium), or compounds, double salts, or physically associated mixtures of these with one or more other acid soluble materials of a substantially water insoluble nature.

By the term "alkaline filler" I also intend to include fibrous material and/or other material such as paper coating constituents or the like containing one or more compounds of the character referred to, such as "old papers" or similar papers, "broke", or the like.

When I use the word "paper" herein, I use it in the broad sense to include products of manufacture of all types and of all weights and thicknesses, which contain as an essential constituent a considerable amount of prepared fibre and which are capable of being produced on a Fourdrinier, cylinder, or other forming, felting, shaping or molding machine.

By the term "wet end of the paper machine" 130

I intend to include those instrumentalities employed in paper manufacture by which and/or in which a relatively concentrated paper mix is diluted, and treated, conveyed or fed up to the point of web-formation such as the mixing box, regulating and proportioning devices, rifflers, troughs, screens, head boxes, inlets, and the like, including also instrumentalities used in the white water cycle.

10 Where I use the expression "soft lumps" I mean lumps which have their origin subsequent to the screening of the stock, being formed in the head box, inlet or the like. These lumps are entirely different, and easily 15 distinguishable by practical paper makers, from slime, i. e. masses of stock usually fermented or decomposed which settle or form on chest and pipe surfaces, and when dislodged work through the screens and on to 20 the wire. Of course, slime also forms in the head box and inlets after the machine has run for a relatively long period of time without wash-up, but the soft lumps I describe are entirely distinct therefrom and form, and 25 start to give trouble, even within as short a time as several hours after the head box and inlet have been thoroughly cleaned.

Where I use the word "casein" herein, I use it in the generic sense to include casein and/or 30 compounds or derivatives thereof.

While I have described in detail the preferred embodiment of my invention, it is to be understood that the details of procedure, the proportions of ingredients, and the arrangement of steps may be widely varied without departing from the spirit of the invention or the scope of the subjoined claims.

I claim:

1. The method of manufacturing paper 40 filled with alkaline filler and containing casein in its furnish, comprising adding to a fibrous mix originally comprising fibrous material, casein bearing constituent, and alum, alkaline filler under conditions favoring the 45 minimizing of time of contact of the constituents of the mix, and thereafter making paper therefrom.

2. The method of manufacturing paper 50 filled with alkaline filler and containing casein in its furnish, comprising adding to a fibrous mix originally comprising fibrous material, casein bearing constituent, and alum, alkaline filler under conditions favoring the 55 minimizing of intimacy and time of contact of the constituents of the mix, and thereafter making paper therefrom.

3. The method of manufacturing paper 60 filled with alkaline filler and containing casein in its furnish, comprising adding to a fibrous mix originally comprising fibrous material, casein bearing constituent, and alum, alkaline filler at the wet end of the paper machine, and thereafter making paper therefrom.

65 4. The method of manufacturing paper

filled with alkaline filler and containing casein in its furnish, comprising adding to a fibrous mix originally comprising fibrous material, casein bearing constituent, and a salt of aluminum, alkaline filler at the wet end of the paper machine, and thereafter making paper therefrom.

5. The method of manufacturing paper 70 filled with alkaline filler and containing casein in its furnish, comprising adding to a fibrous mix originally comprising fibrous material, casein bearing constituent, and a metallic salt, alkaline filler at the wet end of the paper machine, and thereafter making paper 75 therefrom.

6. The method of manufacturing paper 80 filled with alkaline filler and containing casein in its furnish, comprising adding to a fibrous mix originally comprising fibrous material, casein bearing constituent, and acidic material, alkaline filler at the wet end of the paper machine, and thereafter making paper 85 therefrom.

7. The method of manufacturing paper 90 filled with alkaline filler and containing casein in its furnish, comprising adding to a fibrous mix originally comprising fibrous material including old paper stock, casein bearing constituent, and alum, alkaline filler at the 95 wet end of the paper machine, and thereafter making paper therefrom.

8. The method of manufacturing paper 100 filled with alkaline filler and containing casein in its furnish, comprising adding to a fibrous mix originally comprising fibrous material including sulphite pulp and soda pulp and old paper stock, casein bearing constituent, and alum, alkaline filler at the wet end of the paper machine, and thereafter making 105 paper therefrom.

9. The method of manufacturing paper 110 filled with alkaline filler and containing casein in its furnish, comprising adding to a fibrous mix originally comprising fibrous material, casein bearing constituent comprising coated broke, and alum, alkaline filler at the wet end of the paper machine, and thereafter making paper therefrom.

10. The method of manufacturing paper 115 filled with alkaline filler and containing casein in its furnish, comprising adding to a fibrous mix originally comprising fibrous material including old paper stock, casein bearing constituent comprising coated broke, and alum, alkaline filler at the wet end of the paper machine, and thereafter making paper 120 therefrom.

11. The method of manufacturing paper 125 filled with alkaline filler and containing casein in its furnish, comprising adding to a fibrous mix originally comprising fibrous material, casein bearing constituent, and alum, alkaline filler comprising alkaline earth metal compound at the wet end of the paper ma- 130

- chine, and thereafter making paper therefrom.
12. The method of manufacturing paper filled with alkaline filler and containing casein in its furnish, comprising adding to a fibrous mix originally comprising fibrous material, casein bearing constituent, and alum, alkaline filler comprising calcium carbonate at the wet end of the paper machine, and thereafter making paper therefrom. 70
13. The method of manufacturing paper filled with alkaline filler and containing casein in its furnish, comprising adding to a fibrous mix originally comprising fibrous material, casein bearing constituent, and alum, alkaline filler comprising calcium carbonate and magnesium compound at the wet end of the paper machine, and thereafter making paper therefrom. 75
14. The method of manufacturing paper filled with alkaline filler and containing casein in its furnish, comprising adding to a fibrous mix originally comprising fibrous material, casein bearing constituent, and alum, alkaline filler comprising calcium carbonate magnesium hydroxide at the wet end of the paper machine, and thereafter making paper therefrom. 80
15. The method of manufacturing paper filled with alkaline filler and containing casein in its furnish, comprising adding to a fibrous mix originally comprising fibrous material, casein bearing constituent, and sizing, alkaline filler at the wet end of the paper machine, and thereafter making paper therefrom. 85
16. The method of manufacturing paper filled with alkaline filler and containing casein in its furnish, comprising adding to a fibrous mix originally comprising fibrous material, casein bearing constituent, and size precipitated by an excess of alum, alkaline filler at the wet end of the paper machine, and thereafter making paper therefrom. 90
17. The method of manufacturing paper filled with alkaline filler and containing casein in its furnish, comprising adding to a fibrous mix originally comprising fibrous material, casein bearing constituent, and size in an amount insufficient to produce a substantial degree of sizing in the paper precipitated by an excess of alum, alkaline filler at the wet end of the paper machine, and thereafter making paper therefrom. 95
18. That step in the method of manufacturing paper filled with alkaline filler and containing casein in its furnish comprising adding alkaline filler to the paper mix at the wet end of the paper machine. 100
19. The method of manufacturing paper filled with alkaline filler and containing casein in its furnish, comprising adding to a fibrous mix comprising fibrous material and casein bearing constituent, alkaline filler and acidic material at the wet end of the paper machine, and thereafter making paper therefrom. 105
20. The method of manufacturing paper filled with alkaline filler and containing casein in its furnish, comprising adding to a fibrous mix comprising fibrous material and casein bearing constituent, alkaline filler and a metallic salt at the wet end of the paper machine, and thereafter making paper therefrom. 110
21. The method of manufacturing paper filled with alkaline filler and containing casein in its furnish, comprising adding to a fibrous mix comprising fibrous material and casein bearing constituent, alkaline filler and a salt of aluminum at the wet end of the paper machine, and thereafter making paper therefrom. 115
22. The method of manufacturing paper filled with alkaline filler and containing casein in its furnish, comprising adding to a fibrous mix comprising fibrous material and casein bearing constituent, alkaline filler and alum at the wet end of the paper machine, and thereafter making paper therefrom. 120
23. The method of manufacturing paper filled with alkaline filler and containing casein in its furnish, comprising adding to a fibrous mix comprising fibrous material, casein bearing constituent, and sizing, alkaline filler and alum at the wet end of the paper machine, and thereafter making paper therefrom. 125
24. The method of manufacturing paper filled with alkaline filler and containing casein in its furnish, comprising adding to a fibrous mix comprising fibrous material, casein bearing constituent, and rosin size, alkaline filler and alum at the wet end of the paper machine, and thereafter making paper therefrom. 130
25. The method of manufacturing paper filled with alkaline filler and containing casein in its furnish, comprising adding to a fibrous mix comprising fibrous material, casein bearing constituent, and size in an amount insufficient to impart a substantial degree of sizing to the paper, alkaline filler and alum at the wet end of the paper machine, and thereafter making paper therefrom. 135
26. That step in the method of manufacturing paper filled with alkaline filler and containing casein in its furnish comprising adding alkaline filler and alum to the paper mix at the wet end of the paper machine. 140

In testimony whereof I affix my signature.  
HAROLD ROBERT RAFTON.